

# United States Patent Office.

WALDRON J. CHEYNEY, OF WALLINGFORD, AND EMIL F. DIETERICHS,  
OF PHILADELPHIA, PENNSYLVANIA.

*Letters Patent No. 69,315, dated October 1, 1867; antedated September 20, 1867.*

## IMPROVED ARCHITECTURAL PORCELAIN.

The Schedule referred to in these Letters Patent and making part of the same.

### TO ALL WHOM IT MAY CONCERN:

Be it known that we, WALDRON J. CHEYNEY, of Wallingford, Delaware county, and EMIL F. DIETERICH, of the city and county of Philadelphia, both of the State of Pennsylvania, have invented a new and useful improvement in building material, which we call "Architectural Porcelain;" and we do hereby declare that the following is a full and exact description of the same.

Our material may be used for building-blocks, either hollow or solid; pillars or columns, either hollow or solid; cornices and balusters, either hollow or solid; caps, sills, tiles for floors, roofs, and walls, either inside or outside; mouldings, centre-pieces, bath-tubs, wash-stands, basins, urinals, and generally for all articles, either of use or ornament, which are employed in the construction and fitting up of buildings.

Our architectural porcelain is composed of cryolite, or its chemical equivalents, and silica, alone or in combination with the oxide of zinc, the whole fused together in a crucible, and cast in moulds, or pressed or rolled, the choice of either of these modes of production being governed by the form of the article desired.

In making our "architectural porcelain," we have found the following combination and proportions to answer well, (although the oxide of zinc may be omitted, or another metallic oxide substituted for it, or the proportions of the other minerals varied, without material detriment; if the cryolite is materially diminished, an alkali must be added:) Fifty pounds of sand, (silicious,) twenty pounds of cryolite, (powdered,) five pounds of white oxide of zinc.

Having thus described our invention, we claim, and desire to secure by Letters Patent, as a new article of manufacture—

"Architectural porcelain," composed of cryolite, or its chemical equivalents, and silica, alone, or cryolite, or its chemical equivalents, in combination with silica and a metallic oxide, or an alkali, or both, fused and cast in moulds, and pressed or rolled, as above set forth.

WALDRON J. CHEYNEY,  
E. F. DIETERICH.

Witnesses:

GEO. E. BUCKLEY,  
F. B. KENNER.